

# UNITED STATES PATENT OFFICE.

THEODORE D. PALMER, OF NEWARK, NEW JERSEY.

## ART OF TANNING HIDES.

SPECIFICATION forming part of Letters Patent No. 625,411, dated May 23, 1899.

Application filed December 10, 1898. Serial No. 699,019. (No specimens.)

*To all whom it may concern:*

Be it known that I, THEODORE D. PALMER, a citizen of the United States, residing in the city of Newark, county of Essex, and State of New Jersey, have invented a new and useful Improvement in the Art of Tanning Hides, of which the following is a specification.

This invention relates to the art or process of tanning hides and skins to convert them into leather, the object being to provide a process by which the hides can be converted into leather in a very short space of time at a reduced cost and at the same time have the process so arranged that the best results can be had—that is, the finest and best grades of leather may be produced with the least possible cost.

The process of tanning heretofore has been to immerse the hides in a liquor made from bark, wood, or herbs—such as hemlock, oak, quebrachos, gambrie, or canagrie root—containing tannic acid as active agent and certain other substances commonly known as "reds," which are found necessary in tanning. First the solution is weak and is gradually increased in strength until it is thoroughly incorporated within the hide. Sometimes mechanical means are used to agitate the liquor, thus making it more quickly penetrate the hide; but in either case the process is very slow and it takes about four months to produce anything like a properly-tanned hide. Thus a great deal of room and a large number of tubs and considerable handling to do a very little work are necessary and make the process expensive.

The reason why the liquor is so slow in penetrating the hide in the above-described method is the fact that the tanning agents, such as the barks and herbs above referred to, are not thoroughly dissolved and do not impart their full strength until the hides have been in the liquor for a long time. This is shown in all such solutions by a flaky appearance of the liquid caused by the undissolved particles. The method which I adopt, therefore, and which not only quickens the process, but makes better leather, is as follows: I first take the tanning liquor, which is mixed of the usual ingredients, as above described, and to this add a suitable clarifying agent, such as borax or other ingredient

having a like chemical action, in sufficient quantities to form a chemical combination between the tannins, reds, and gums of the liquor, forming a solution quite clear of any undissolved particles. The hide is then prepared by any of the well-known processes and is then immersed in the clarified liquor. The liquor being thoroughly clarified, as above described, will penetrate the hide very quickly and produce the desired result in a very short space of time, probably one-tenth of the time required by the usual and slower method. When the hide is thoroughly filled with the clarified liquor, (or has in the judgment of the operator taken up sufficient of the tanning matter to produce the class of leather he desires to make, which will be in about five to six days for upper-leather and eight to ten days for sole-leather,) it is immersed in a bath of weak acid or other well-known reacting agents to precipitate again the tanning liquor in the hide and render it permanent there. This is shown by water only, and not tan liquor, being expelled from the hide when being squeezed or pressed. (A weak oxalic-acid bath with alum or salt has been found most satisfactory for this.) After the latter process of precipitating in the hide all of the tanning material absorbed by it in the tanning-bath the hide is left clear without the necessity of scouring and loss attending the same and is generally lighter and more uniform in color.

I have described above that the liquors should be entirely clear and then that the tannings should be entirely reprecipitated in the hide. These are the points which in practice show the best results and greatest economy, though the process is applicable when these points are only approximately reached.

The principal advantages are saving in the tan liquor, the more rapid manner in which the work can be done, and the effect upon the leather, which renders it of a superior grade. With my improved process an ordinary fifty-pound hide can be treated in about five days and will produce the finest grade of rough or upper leather, and the more heavy sole-leather hides can be treated in about eight days, thus reducing the labor necessary in handling and producing much better leather.

Having thus described my invention, what I claim, and desire to secure by Letters Patent of the United States, is—

1. The process herein described for tanning leather which consists of adding a suitable clarifying agent as herein described, to clarify the tanning liquor and immersing the hide therein, after which it is submitted to an acid-bath to reprecipitate the liquor in the hide, substantially as described.
2. The art of tanning hides or skins by

clarifying the tanning liquor, and reprecipitating it when in the hide, substantially as set forth.

In testimony that I claim the foregoing <sup>15</sup> specification I have hereunto set my hand this 18th day of August, 1897.

THEODORE D. PALMER.

In presence of—  
C. L. MALCOLM,  
J. H. BELL.